

**[54] STATIC CHARGE-PREVENTED  
PHOTOGRAPHIC LIGHT SENSITIVE  
ELEMENT**

[76] Inventors: **Takayuki Inayama; Wataru Ueno; Nobuo Tsuji**, all of 210 Nakanuma, Minami Ashigara-Machi, Ashigara Kamigun, Kanagawa, Japan

[22] Filed: **Feb. 8, 1972**

[21] Appl. No.: **224,598**

**[30] Foreign Application Priority Data**

Feb. 8, 1971 Japan..... 46/5062

[52] U.S. Cl..... **96/87 A, 96/67, 96/114.2**

[51] Int. Cl..... **G03c 1/82**

[58] Field of Search..... **96/87 A, 114.2**

**[56] References Cited****UNITED STATES PATENTS**

|           |        |                  |         |
|-----------|--------|------------------|---------|
| 2,461,474 | 2/1949 | Kaszuba.....     | 96/87 A |
| 3,457,076 | 7/1969 | Yano et al. .... | 96/87 A |

Primary Examiner—Ronald H. Smith

Attorney—Richard C. Sughrue et al.

**[57] ABSTRACT**

A static charge-prevented photographic light sensitive element using an antistatic agent in combination with a dichlorophenylphenylsulfone. The combination can reduce the surface resistivity very more than in the case where the antistatic agent is used alone.

**11 Claims, No Drawings**

# STATIC CHARGE-PREVENTED PHOTOGRAPHIC LIGHT SENSITIVE ELEMENT

## BACKGROUND OF THE INVENTION

## 1. Field of the Invention

This invention relates to static charge-prevented photographic light sensitive elements. More particularly, this invention relates to employment of a dichlorophenylphenylsulfone in combination with an antistatic agent to significantly reduce the surface resistivity and thereby to impart the static charge preventing effect.

## 2. Description of the Prior Art

In the manufacture and use of photographic films, when the films are statically charged too much an electric discharge will occur between the charged films and neighboring conductors when the films are exposed thereto, resulting in the accident of static marks. The accident of static marks also occurs when the surface of the base is stripped from the emulsion surface upon rolling back a film. 15 20

In an attempt to prevent a photographic film from being statically charged, antistatic agents of varied types have been used heretofore. It is known that the higher the concentration of the antistatic agent is, the lower the surface resistivity becomes. Therefore, the antistatic agent is used in such an amount that the surface resistivity may become approximately from  $10^{11}$  to  $10^{12}$  ohms. However, when an excessive amount of an antistatic agent is used, the photographic emulsion undergoes a deteriorating influence or adhesion interference, the application of such an excessive amount of the antistatic agent being impractical in most cases.

## DESCRIPTION OF THE INVENTION

We have now found that the above-described various defects can be eliminated by incorporating both a dichlorophenylphenylsulfone of the invention and an antistatic agent into at least one of auxiliary layers in a photographic film, for example, an anticurl layer or antihalation layer, or by applying them onto at least one of the surfaces of said layers or of a support. Thus, the present invention provides an excellent method whereby the surface resistivity can be reduced very much more than in the case where the antistatic agent is used alone. The method of the invention is extremely effective even when carried out under low humidity and its static-charge preventing effect is not changed with the passage of time. Furthermore, the dichlorophenylphenylsulfone is inert to photographic emulsions and exerts no deteriorating influence upon the photographic properties thereof.

The dichlorophenylphenylsulfones used according to the present invention may be represented by the following general formula 55



Examples of such compounds include 2,4-dichlorophenylphenylsulfone, 2,5-dichlorophenylphenylsulfone, 3,4-dichlorophenylphenylsulfone, and the like.

Reference will now be made to the method of synthesizing these dichlorophenylphenylsulfones.

2

The dichlorophenylphenylsulfones used according to the invention can be easily prepared by the Friedel-Craft reaction of the corresponding dichlorobenzenesulfonylchloride with benzene in the presence of iron chloride. The melting points of some dichlorophenylphenylsulfones are as follows.

|    |                                 | M.P.     |
|----|---------------------------------|----------|
|    | 2,4-dichlorophenylphenylsulfone | 97°-98°C |
|    | 2,5-dichlorophenylphenylsulfone | 147°C    |
| 10 | 3,4-dichlorophenylphenylsulfone | 125°C    |

Synthesis examples of these compounds are described in detail in U.S. Pat. No. 2,224,964 (1939).

The antistatic agents usable in the present invention 15 include known or commercially available antistatic agents having the following formulas, but are not limited to these compounds.

### cationic antistatic agent



### **anionic antistatic agent**



### amphoteric antistatic agent



When these compounds are applied to a photographic light sensitive element, they should not exert any deteriorating influence upon photographic properties such as sensitivity, fog, or gradation.

When the method of the invention is applied to the back of a photographic film base, both of the two components of the invention may be coated on its surface by spraying with the aid of an organic solvent or by dipping the surface in a solution of the components in the organic solvent, followed, in either case, by drying. The two components of the invention may also be used together with a binder such as gelatin, polyvinyl alcohol, polycarbonate or cellulose acetate.

electrodes was made of stainless steel) and reading 1-minute value of an insulation tester (Type M - V, provided by Takeda Riken Ind. Co., Ltd.). The static charge generation test was conducted by the method in which an unexposed film is placed with the back surface below on a rubber sheet, and the stack adhered by pressuring with a rubber roller and thereafter stripped to generate static marks.

The temperature-humidity conditions used for the measurement was 23°C - 65 percent R.H. or 23°C - 25 percent R.H.

The moisture adjustment of test pieces was carried out under the above described conditions for about a half day.

15

#### EXAMPLE 1

An antistatic solution of the following formulation was applied by the dipping method onto a polyethylene terephthalate film 0.1 mm thick and immediately thereafter dried at 120°C. for 30 minutes using an air bath.

#### FORMULATION OF THE ANTISTATIC SOLUTION

10 wt. percent solution of 2,5-dichlorophenylphenylsulfone according to the invention in acetone.

Quantities added specified in Table 1.

10 wt. percent methanolic solution of an antistatic agent.

Quantities added specified in Table 1.

A binder solution (5 wt. percent solution of cellulose triacetate in

92 : 8, by weight, of methylene chloride : methanol) - 12 g.

Phenol - 2 g.

Tetrachloroethane - 8 g.

Ethylene chloride - 85 g.

Methanol - 5 g.

The surface resistivity is shown in Table 1.

TABLE 1

| Test piece number | Compound of the invention       | Quantities, percent* | Antistatic agent                  | Quantities, percent* | Surface resistivity (Ω)          |
|-------------------|---------------------------------|----------------------|-----------------------------------|----------------------|----------------------------------|
| 1.                |                                 | 0                    |                                   |                      | 0 More than $1 \times 10^{16}$ . |
| 2.                | 2,5-dichlorophenylphenylsulfone | 5                    |                                   |                      | 0 Do.                            |
| 3.                | do                              | 10                   |                                   |                      | 0 Do.                            |
| 4.                |                                 | 0                    | Alkyl phosphoric acid ester salts | 5                    | $2 \times 10^{12}$ .             |
| 5.                | 2,5-dichlorophenylphenylsulfone | 5                    | do                                | 5                    | $8 \times 10^{10}$ .             |
| 6.                |                                 | 0                    |                                   |                      | $3 \times 10^{15}$ .             |
| 7.                | 2,5-dichlorophenylphenylsulfone | 5                    | Same as above                     | 5                    | $5 \times 10^{12}$ .             |
| 8.                | do                              | 0                    |                                   | 5                    | $5 \times 10^{12}$ .             |
| 9.                | 2,5-dichlorophenylphenylsulfone | 10                   | do                                | 10                   | $7 \times 10^{10}$ .             |

\*The ratio in percent of the active ingredient to the binder.

The present invention may be used for the purpose of static charge prevention in films or moulded materials comprising cellulose esters, polyesters, polystyrenes or polycarbonates.

The invention will be further illustrated by the following examples.

In these examples, the surface resistivity was determined by interposing a test piece between brassy electrodes of 10 cm. in length spaced by 0.14 cm. (the part of the electrodes at which the test piece contacts the

60 As is evident from the above-described Table 1, the combination of 2,5-dichlorophenylphenylsulfone with an antistatic agent can reduce the surface resistivity very much more than in the case where the antistatic agent is used alone, thereby showing an excellent synergistic effect.

#### EXAMPLE 2

The procedure as described in Example 1 was followed using an antistatic solution of the same formula-

tion as in Example 1 but using sodium nonylphenoxypropanesulfonate as the antistatic agent. The surface resistivity at 25 percent R.H. is shown in Table 2.

4. A static charge-prevented photographic light sensitive element as claimed in claim 1 wherein the support in the element is made of a cellulose ester, polystyrene, or polycarbonate.

TABLE 2

| Test piece number | Compound of the invention       | Quantities, percent* | Antistatic agent                    | Quantities, percent* | Surface resistivity (Ω)      |
|-------------------|---------------------------------|----------------------|-------------------------------------|----------------------|------------------------------|
| 10                |                                 | 0                    | Sodium nonylphenoxypropanesulfonate | 5                    | $1 \times 10^{14}$           |
| 11                | 2,5-dichlorophenylphenylsulfone | 5                    | Same as above                       | 0                    | More than $1 \times 10^{16}$ |
| 12                | do                              | 5                    | do                                  | 5                    | $2 \times 10^{12}$           |

\*The ratio in percent of the active ingredient to the binder.

As is evident from the above-described Table 2, the present combination of 2,5-dichlorophenylphenylsulfone with an antistatic agent can reduce the surface resistivity very much more than in the case where the antistatic agent is used alone, thereby showing a significant static charge-preventing effect.

Furthermore, in the above-described static-charge preventing processing, a silver chlorobromide photographic emulsion for printing use containing 30 mole percent of silver bromide was applied onto the opposite surface of the film.

In the static charge generation test, at 25 percent R.H., little generation of static marks was observed with the films processed according to the invention but remarkable generation thereof with the films not processed in accordance with the present invention was observed.

This invention has been described in considerable detail with particular reference to preferred embodiments thereof, but it will be understood that variations and modifications can be effected within the spirit and scope of the invention as described hereinabove and as defined in the appended claims.

We claim:

1. A static charge-prevented photographic light sensitive element, which comprises a support having coated thereon, a silver halide light-sensitive emulsion layer which is characterized by using an antistatic agent in combination with a dichlorophenylphenylsulfone represented by the following general formula



said antistatic agent and said dichlorophenylphenylsulfone being incorporated, in combination, into at least one auxilliary photographic layer maintained on said support.

2. A static charge-prevented photographic light sensitive element as claimed in claim 1 wherein said dichlorophenylphenylsulfone is selected from the group consisting of 2,4-, 2,5- and 3,4-dichlorophenylphenylsulfones.

3. A static charge-prevented photographic light sensitive element as claimed in claim 2 wherein said dichlorophenylphenylsulfone is 2,5-dichlorophenylphenylsulfone.

5. A static charge-prevented photographic light sensitive element as claimed in claim 4 wherein the support in the element is a polyethylene terephthalate film.

6. A static charge-prevented photographic light-sensitive element as claimed in claim 1 wherein said antistatic agent is a cationic antistatic agent.

7. A static charge-prevented photographic light-sensitive element as claimed in claim 6, wherein said cationic antistatic agent is a member selected from the group consisting of those compounds listed below having the following formulae (I), (II), (III), and (IV).



55 8. A static charge-prevented photographic light-sensitive element as claimed in claim 1 wherein said antistatic agent is an anionic antistatic agent.

9. A static charge-prevented photographic light-sensitive element as claimed in claim 8, wherein said anionic antistatic agent is a member selected from the group consisting of those compounds listed below having the formulae (V), (VI), (VII), (VIII), (IX) or (X):



(VII)



(VIII)



(IX)



(X)



(XI)



(XII)



(XIII)



\* \* \* \* \*

10. A static charge-prevented photographic light-sensitive element as claimed in claim 1 wherein said antistatic agent is an amphoteric antistatic agent.

11. A static charge-prevented photographic light-sensitive element as claimed in claim 10, wherein said amphoteric antistatic agent is a member selected from the group consisting of those compounds listed below having the following formulae (XI), (XII), (XIII), (XIV) or (XV):